# EUROPEAN PATENT SPECIFICATION

(11) **EP 0 228 489 B1**
(45) Date of publication and mention of the grant of the patent: **14.06.1989**
(21) Application number: 85309479.5
(22) Date of filing: 24.12.1985
(51) Int. Cl.: C10M 135/04, C07C 148/00, C10N 30/06

(54) **Sulfurized olefin process and products thereof, and compositions containing such olefins and their production**
Verfahren zur Herstellung von sulfurierten Olefinen und Produkte davon und diese Olefine enthaltende Zusammensetzungen und deren Herstellung
Procédé pour la sulfuration d'oléfines et leurs produits, et compositions contenant ces oléfines et leur production

(43) Date of publication of application: 15.07.1987
(73) Proprietor: ETHYL PETROLEUM ADDITIVES, INC., Baton Rouge Louisiana 70801 (US)
(72) Inventor: Griffin, Paul G., Collinsville Illinois 62234 (US); Yuk-Lun Lam, William, Ballwin Missouri 63021 (US)
(74) Representative: Bizley, Richard Edward

(56) References cited:
- US-A- 4 188 297
- US-A- 4 204 969

## Description

Sulfurized olefins are well-known additives in lubricating oil, cutting oil and the like. Kimball, U.S. Pat. No 2 249 312, describes such a product. Eby, U.S. Pat. No 2 708 199, describes a similar product in which a sulfur halide is reacted with an olefin using a lower alkanol promoter to obtain an intermediate which is reacted with an alkali or alkaline earth metal polysulfide. Myers, U.S. Pat. No 3 471 404, describes a product in which sulfur monochloride is reacted with olefin to obtain an intermediate which is reacted with sulfur and alkali metal sulfide at a critical ratio of 1.8-2.2 gram moles of metal sulfide per gram mole of sulfur. This material is then refluxed for 1-24 hours with aqueous alkali metal hydroxide. In U.S. 4 204 969, an effective sulfurized olefin is made by reacting sulfur monochloride with an olefin in the presence of a lower alkanol promoter to obtain an adduct which is reacted with sodium sulfide and sulfur in aqueous alkanol.

U.S. 4 188 297 discloses a method for making a lubricating additive in which an olefinically unsaturated hydrocarbon is reacted with elemental sulfur and a mercaptan.

According to the present invention, a sulfurized olefin having improved solubility especially in alpha-olefin oligomer lubricating oil is made by a process comprising:
(a) reacting a sulfur halide selected from SCI₂, S₂CI₂ and mixtures thereof with an aliphatic monoolefin containing 3-6 carbon atoms to produce an adduct;
(b) reacting said adduct with sulfur, Na₂S in an amount of from 0.5 to 2.0 gram mole per gram mole of sulfur chloride, an alkyl mercaptan containing 1-12 carbon atoms and from 0 to 0.5 gram mole NaSH per mole of sulfur halide in an aqueous alcohol medium at a temperature of from 50_{°}C up to reflux to form said sulfurized olefin;
(c) recovering said sulfurized olefin from the aqueous alcohol medium.

Although a useful product can be obtained using either SC1₂ or S₂Ct₂, superior results were obtained with S₂C[₂ so this sulfur halide is most preferred.

The olefins used are the monoethylenically unsaturated aliphatic hydrocarbons referred to as aliphatic monoolefins containing 3 to 6 carbon atoms.

Although a useful product can be obtained using either S01₂ or S₂Ct₂, superior results were obtained with S₂CI₂ so this sulfur halide is most preferred.

Useful olefins are the monoethylenically unsaturated aliphatic hydrocarbons referred to as aliphatic monoolefins containing 3 to 6 carbon atoms. These include 1-butene, 2-butene, isobutene, 1-pentene, 2-pentene, 2-methyl-1-butene, 3-methyl-1-butene, 2-methyl-2-butene, 1-hexene, 2-hexene, 3-hexene, 2-methyl-1-pentene, 2-methyl-2-pentene, 2-ethyl-2-butene and the like including mixtures thereof.

Preferably the olefins are branched-chain olefin such as isobutene, 2-methyl-1-butene, 2-methyl-2-butene, 2-methyl-2-pentene and the like. More preferably the ethylenic double bond adjoins a tertiary carbon atom such as isobutylene, the most preferred olefin.

The first stage reaction is preferably conducted by adding the olefin to sulfur monochloride. The olefin can be added as a gas or liquid. Preferably it is added beneath the surface of the sulfur monochloride as a liquid.

In practice the olefin is added until the reaction with the sulfur monochloride stops as indicated by loss of exotherm. An amount of 0.75-3.0 gram moles of olefin for each 0.3-0.75 gram mole of sulfur monochloride usually suffices. A preferred amount is 1.5-2.0 gram moles of olefin per gram mole of sulfur monochloride.

The reaction between sulfur monochloride and olefin will proceed without adding an alcohol promoter, and since alcohol will tend to cause corrosion of metal equipment, it is not a highly preferred method of conducting the first stage. The use of an alcohol promoter, however, is included in one embodiment of the invention. Lower alcohol promoters which can be used in the first stage contains from 1 to 4 carbon atoms. Typical examples are methanol, ethanol, n-propanol, isopropanol, isobutanol, tert-butanol and the like. A preferred promoter is methanol. The amount of alcohol promoter is preferably 0.001 to 0.3 gram moles for each 0.3-0.75 gram mole of sulfur monochloride.

The first stage reaction can be conducted at any temperature high enough to cause the reaction to proceed, but not so high as to cause decomposition of the reactants or products. A useful range is 30_{°}-100_{°}C. A more preferred range is 40_{°}-75_{°}C and a most preferred range is 50_{°}-60_{°}C.

The first stage reaction should be conducted for a time sufficient to complete the reaction between the sulfur chloride and olefin. This time is controlled by the rate at which heat can be removed. Olefin feed rate is preferably controlled to hold the temperature within the desired range. When the sulfur chloride has been consumed the temperature will drop. External heat may be added to continue the reaction for a further time, but this does not appear to be necessary. The overall time required to complete the reaction depends upon the scale of the process and can vary from a few minutes up to 12 or more hours. The time is not critical.

During the first stage reaction HCI gas is evolved so means should be provided to scrub the vent gas from the reactor to remove HCI prior to releasing it to the atmosphere.

In the second stage reaction, adduct from the first stage is reacted with sodium sulfide, sulfur, alkyl mercaptan and optionally sodium hydrosulfide in an aqueous alcohol reaction medium. The second stage is preferably carried out by charging aqueous sodium hydrosulfide, sodium hydroxide, water, alcohol and elemental sulfur flowers or powdered sulfur to a reactor and then adding the adduct and alkyl mercaptan to this at reaction temperature. The NaSH and NaOH react to form sodium sulfide. Excess NaSH remains.

The sodium sulfide may be obtained from any of a number of sources. For example, it can be made by mixing approximately equal mole amounts of sodium hydrosulfide and sodium hydroxide. If hydrogen sulfide is available, it can be adsorbed in aqueous NaOH to form a solution of sodium sulfide and/or sodium hydrosulfide depending upon the amount of hydrogen sulfide absorbed. Whatever the source, the resulting solution should be adjusted with either NaOH, NaSH or H₂S so that the resulting solution consists mainly of sodium sulfide and optionally sodium hydrosulfide with little or no free sodium hydroxide.

The amount of sodium sulfide can vary from 0.5-2.0 gram mole for each gram mole of sulfur chloride used in the first reaction stage. Preferably the amount of sodium sulfide is 0.5-1.0 gram mole per mole of sulfur chloride and most preferably 0.6-1.0 gram mole per gram mole sulfur chloride.

Presence of NaSH is optional. Use of up to 0.5 gram moles of NaSH per mole of S₂CI₂ has given satisfactory results. A preferred amount is 0.1-0.3 gram moles and most preferably 0.25 moles per mole of S₂CI₂.

The amount of water can vary widely without detrimental effect. Good results can be obtained using 10-20 gram moles of water per gram mole of sodium sulfide. This includes water added as such, water in aqueous reactants and water which might be formed by reaction of hydrogen sulfide or sodium hydrosulfide with sodium hydroxide in forming sodium sulfide solution.

Alcohol is required in the second stage reaction. Preferably, these are lower alcohols containing 1-4 carbon atoms such as methanol, ethanol, n-propanol, n-butanol, isobutanol, tert-butanol and the like, including mixtures thereof. The preferred alcohol is isopropanol either alone or mixed with other alkanols such as tert-butanol.

The amount of alcohol can likewise vary over a wide range. A useful range is 0.25-0.75 parts by weight per each part by weight of water. A more preferred range is 0.4-0.6 parts by weight alcohol per each part by weight water.

The alkyl mercaptan can be added separately to the aqueous alcohol reaction medium or it can be mixed with the first stage adduct and the mixture added to the aqueous alcohol containing the sodium sulfide and sulfur. When added separately it is preferred that it be added concurrently with the first stage adduct to the aqueous alcohol containing the sodium sulfide and sulfur. Sequential addition can be used but it is not preferred.

The alkyl mercaptans used are those in which the alkyl group contains 1 to 12 carbon atoms. Representative example of these are methyl mercaptan, ethyl mercaptan, n-propyl mercaptan, i-propyl mercaptan, n-butyl mercaptan, isobutyl mercaptan, sec-butyl mercaptan, tert-butyl mercaptan, n-pentyl mercaptan, isopentyl mercaptan, tert-pentyl mercaptan, 2-ethyl hexyl mercaptan, n-octyl mercaptan, 1-methyl-heptyl mercaptan, 1-ethyl-decyl mercaptan and the like including mixtures thereof.

Of the foregoing the more preferred mercaptans are the tert-alkyl mercaptans. Of these the more preferred are the tert-alkyl mercaptans containing 4-8 carbon atoms. The most preferred alkyl mercaptan is tert-butyl mercaptan.

The amount of alkyl mercaptan can vary over a wide range. A useful range in which to test is 0.05 to 0.8 moles for each mole of sulfur monochloride used in the first stage. A preferred range is 0.08 to 0.5 moles of alkyl mercaptan per mole of sulfur monochloride and a more preferred range is 0.1 to 0.4 moles per mole of sulfur monochloride. The most preferred amount of alkyl mercaptan is 0.25 to 0.35 moles per mole of sulfur monochloride.

The preferred amount of sulfur added is 0-0.3 gram atom for each gram mole of S₂CI₂. More preferably, 0.05-0.15 gram atom of sulfur and most preferably 0.0-0.15 gram atom are used per gram mole of S_{P}OI₂.

In a preferred mode of operation the mixture of sodium sulfide, sulfur and aqueous alkanol is stirred and heated to reaction temperature and then the adduct and alkyl mercaptan are added to it. However, the reaction can be carried out in other ways such as by adding the sodium sulfide, sulfur, alkyl mercaptan and aqueous alkanol mixture to the adduct or by mixing everything together and heating the mixture.

Preferred second stage reaction temperature is 50_{°}C up to reflux temperature. A more preferred 10 reaction temperature is 75-85°C.

After the adduct and alkyl mercaptan have been added to the sodium sulfide/sulfur/aqueous alkanol mixture, which is usually completed in 1-8 hours, the mixture is preferably heated to reflux just below for 2-8 hours to assure completion of the reaction.

A very convenient way in which to make an effective sulfurized isobutylene is to base the amount of Na₂S and NaSH (or NaOH plus NaSH or NaOH plus H₂S), sulfur and tert-butyl mercaptan on the weight of S₂CI₂ - isobutylene adduct. Following this procedure the Kg of Na₂S, NaSH, sulfur and tert-butyl mercaptan per each 100 Kg of sulfurized isobutylene is preferably 15-45:0-12:0-7.5:3-20:100, more preferably 20-35:2-10:1-6:4-18:100 and most preferably 25-30:4-8:2-5:5-15:100. After reaction of the adduct with sodium sulfide, sodium hydrosulfide, alkyl mercaptan and sulfur the product is recovered by conventional methods such as removing alkanol, water washing and filtering.

The following example illustrates the manner of making the sulfurized olefin.

### EXAMPLE 1

A sulfurized isobutylene adduct was made by adding isobutylene to sulfur monochloride at 50-65°C until reaction stopped. In a separate vessel was placed 177.9g aqueous alcohol (64.7 wt% isopropanol, 13.8 wt% tert-butanol, 20.3 wt% water), 23.4g water, 240.4g 29.09% aqueous NaSH solution (0.9 moles), 76.2g 81.6g 50% aqueous NaOH solution (0.95 moles) and 12.3g (0.38 moles) sulfur. This was stirred at 75_{°}C while 255.3g of the above adduct and 32.0g tart-butyl mercaptan (0.36 moles) were concurrently added dropwise over a two hour period. Heat was continued at reflux for three hours and then solvent alcohol was distilled out up to 90°C. Vacuum was applied to remove more solvent. Heat was stopped and when the mixture cooled to 65_{°}C the mixture was washed with water. The aqueous brine layer was removed and the organic layer was stripped of volatiles under vacuum at 100-110_{°}C for one hour and then filtered a second time giving a clear amber product which analyzed 47.7 weight percent sulfur.

### EXAMPLE 2

In a reaction vessel was placed 188.4g aqueous alcohol (same as in Example 1), 23.3g water 246.0g 29.09 wt% aqueous NaSH (1.27 moles), 78.0g 50% aqueous NaOH (0.98 moles) and 6.1g sulfur (0.44 moles). This mixture was stirred and heated to 75_{°}C and then 270.0g of the sulfurized isobutylene adduct described in Example 1 was fed to the reaction mixture together with 33.9g tert-butyl mercaptan over a two hour period at 75_{°} to reflux. Reflux was continued for three hours and then solvent was distilled out up to liquid temperature of 90_{°}C. Vacuum was applied and heating stopped. When the temperature dropped to 65_{°}C water was added to wash the organic phase. The lower aqueous brine layer was removed. The organic phase was stripped under vacuum at 100-110°C for one hour and then filtered using a filter aid. Product analyzed 43.6 weight percent sulfur.

### EXAMPLE 3

In a reaction vessel was placed 100.41 g of a 34.3 wt% aqueous solution NaSH containing 1.03 wt% Na₂S, 37.27g of a 50 wt% aqueous NaOH solution, 4.0g of sulfur, 43.64g water and 86.19g of a mixture of 65.17 wt% isopropanol, 16.89 wt% tertbutanol and the balance water. this was stirred and heated to 75°C at which time 133.47g of S₂CI₂ - isobutylene adduct made by adding isobutylene to S₂Cl₂ at 60°C to the point where no further isobutylene would react was added concurrently with 6.66g tert-butyl mercaptan over a two hour period. Stirring was continued at reflux (about 80_{°}C) for three hours at which time alcohol-water was distilled out up to 90_{°}C. Vacuum was applied and distillation continued until 70_{°}C liquid temperature at a vacuum of twenty-four inches Hg. The mixture was then water washed at 70_{°}C. Wash water was drained off and 1% Dicalite filter aid added. The mixture was stirred at 100-105_{°}C at 28" Hg vacuum for one hour and then filtered. Product analyzed 48.8 weight percent sulfur.

### EXAMPLE 4

Another product was made following the same procedure as Example 3 except using 98.27g 34.3 wt% aqueous NaSH, 36.48g 50wt% aqueous NaOH, 2.95g sulfur, 42.70g water, 84.66g of same aqueous isopropanol tert-butanol solution 16.33g tert-butyl mercaptan and 130.64g S₂CI₂ - isobutylene adduct. The product analyzed 46.4 weight percent sulfur.

### EXAMPLE 5

This example followed the same procedure as Example 3 except using 94.85g 35.04 wt% aqueous NaSH, 35.96g 50 wt% aqueous NaOH, 6.22g sulfur, 29.77g water, 99.83g 56.39 wt% isopropanol - 13.85 wt% tert-butanol - water solution, 16.21g tert-butyl mercaptan and 129.70g S₂CI₂ - isobutylene adduct. The product analyzed 48 weight percent sulfur.

The sulfurized olefins are especially useful in lubricating oil formulations used in gear applications. The base oil may be a mineral oil or a synthetic oil. Useful synthetic oils include olefin oligomers such as decene trimer, tetramer and pentamer made by oligomerizing 1-decene using a BFa catalyst. Useful olefin oligomers can be made using other catalysts such as the aluminum alkyl Ziegler catalyst. Likewise, other olefins can be used such as Cs-₁₄ 1-olefins.

Synthetic alkylbenzenes can also be used such as di-dodecylbenzene and the like.

Synthetic ester lubricating oil can also be employed such as the alkyl esters of dicarboxylic acid (e.g. di-2-ethylhexylsebacate), fatty acid esters of polyols (e.g. trimethylolpropane, tripelargonate) or complex esters of alkanols, alkane, polyols and carboxylic or polycarboxylic acid.

In this use the sulfurized olefin is added in an amount sufficient to improve the EP property of the lubricant. An amount of 0.1 to 10.0 wt % is usually sufficient.

Fully formulated gear lubricants include other conventional additives which perform various functions. Examples of such other additives are corrosion inhibitors for ferrous and non-ferrous metals such as tetrapropenyl succinic acid and bis-(2,5-alkyldithia)-1,3,4-thiadiazoles. Antiwear additives such as alkyl or aryl phosphonates, phosphite, thiophosphates, dithiophosphates, and phosphoric acids. Also zinc dialkyl or diaryl dithiophosphate, chlorinated hydrocarbons, sulfurized fatty esters and amines.

Tests have been conducted which demonstrate the EP effectiveness of the sulfurized olefin.

The tests were conducted in SAE 90 mineral oil. The first was a 4-ball weld test (ASTM D2783) in which a steel ball is rotated in loaded contact with three fixed balls. The maximum load without weld is recorded as the pass load.

The test additive was blended in the base oil at a concentration which imparted 1.0 weight percent sulfur to the oil. Results obtained were as follows:

In another standard test the present additive was used as a component in a formulated gear oil. The test was an L-42 High Speed Axle Test. Using the additives of Example 1 or 2 gave a gear oil which passed the test.

The mercaptan-capped sulfurized olefins of this invention have been found to be much more soluble in hydrogen-treated mineral oil and alpha-olefin oligomer synthetic lubricating oil compared to the same sulfurized olefin made without mercaptans. In the first comparison blends are made at 4.0 weight percent sulfurized olefin in a hydrotreated base oil, a hydrocracked base oil an alpha-decene oligomer. The blends were rated as clear or cloudy. The results were as follows:

Further solubility tests were conducted to determine the solubility limits of the different additives in a SAE 90W alpha-decene oligomer. The following table gives the maximum concentration for clear solution and concentration at cloudy mixture:

These results show the improvement in solubility in a synthetic alpha-olefin oligomer gear oil base stock due to use of the alkyl mercaptan.

## Claims

1. A process for making a sulfurized olefin having improved solubility in lubricating oil said process comprising
(A) reacting a sulfur halide selected from S₂CI₂ and SCI₂ with an aliphatic monoolefin containing 3-6 carbon atoms to produce an adduct
(B) reacting said adduct with sulfur, Na₂S in an amount of from 0.5 to 2.0 gram mole per mole of sulfar chloride, an alkyl mercaptan containing 1-12 carbon atoms and from 0-0.5 gram mole NaSH per mol sulfur halides in an aqueous alcohol medium at a temperature of 50_{°}C up to reflux to form said sulfurized olefin
(C) recovering said sulfurized olefin from said aqueous alcohol medium.

2. A process as claimed in Claim 1 in which said sulfur halide is S₂Ci₂.

3. A process as claimed in Claim 2 in which said monoolefin is a branched chain monoolefin having 4 to 6 carbon atoms.

4. A process as claimed in Claim 3 in which said monoolefin is isobutylene.

5. A sulfurized olefin useful as an extreme pressure additive in lubricating oil having improved solubility, said sulfurized olefin being the product made by a process comprising:
(A) reacting a sulfur halide selected from S₂C1₂ and SCI₂ with an aliphatic monoolefin containing 3-6 carbon atoms to produce an adduct
(B) reacting said adduct with sulfur, Na₂S in an amount of from 0.5 to 2.0 gram mole per mole of sulfar chloride, an alkyl mercaptan containing 1-12 carbon atoms and from 0-0.5 grams NaSH per mole sulfur halide in an aqueous alcohol medium at a temperature of 50°C up to reflux to form said sulfurized olefin
(C) recovering said sulfurized olefin from said aqueous alcohol medium.

6. A sulfurized olefin as claimed in Claim 5 and further defined by the features of any one or more of claims 2 to 4.

7. A lubricating oil composition comprising a major amount of an oil of lubricating viscosity containing a minor extreme pressure improving amount of a sulfurized olefin as claimed in claim 5 or claim 6.

8. A lubricating oil composition as claimed in Claim 7 in which said olefin is isobutylene, said sulfur halide is S₂C]₂ and said alkyl mercaptan is tert-butyl mercaptan.

9. A process for producing a composition comprising blending into a base oil or hydrocarbon fluid a sulfurized olefin as claimed in Claim 5 or Claim 6 so as to produce either a composition as claimed in Claim 7 or an additive package or concentrate in which the amount of said olefin exceeds said minor extreme pressure improving amount, said additive package thereafter being suitable for further dilution with lubricating oil to produce a lubricating oil composition having pressure-resisting properties.

## Patentansprüche

1. Verfahren zur Herstellung eines sulfurierten Olefins mit verbesserter Löslichkeit in einem Schmieröl, bei dem man:
(A) ein Schwefelhalogenid, ausgewählt aus S₂CI₂ und SCI₂ mit einem aliphatischen Monoolefin, das 3 bis 6 Kohlenstoffatome enthält, zur Herstellung eines Adduktes umsetzt,
(B) das Addukt mit Schwefel, Na₂S in einer Menge von 0,5 bis 2 Gramm-Mol pro Mol Schwefelchlorid, einem Alkylmercaptan, enthaltend 1 bis 12 Kohlenstoffatome und 0 bis 0,5 Gramm-Mol NaSH pro Mol Schwefelhalogenide in einem wäßrigen Alkoholmedium bei einer Temperatur von 50_{°}C bis zu Rückfluß zur Bildung des sulfurierten Olefins umsetzt.
(C) das sulfurierte Olefin aus dem wäßrigen Alkoholmedium abtrennt.

2. Verfahren nach Anspruch 1, bei dem das Schwefelhalogenid S₂CI₂ ist.

3. Verfahren nach Anspruch 2, bei dem das Monoolefin ein verzweigtkettiges Monoolefin mit 4 bis 6 Kohlenstoffatomen ist.

4. Verfahren nach Anspruch 3, bei dem das Monoolefin Isobutylen ist.

5. Sulfuriertes Olefin, brauchbar als Hochdruckadditiv in Schmieröl mit verbesserter Löslichkeit, wobei das sulfurierte Olefin das Produkt eines Verfahrens ist, bei dem man:
(A) ein Schwefelhalogenid, ausgewählt aus S₂C[₂ und SCI₂, mit einem aliphatischen Monoolefin, enthaltend 3 bis 6 Kohlenstoffatome, zur Herstellung eines Adduktes umsetzt,
(B) das Addukt mit Schwefel, Na₂S in einer Menge von 0,5 bis 2 Gramm-Mol pro Mol Schwefelchlorid, einem Alkylmercaptan, enthaltend 1 bis 12 Kohlenstoffatome und 0 bis 0,5 Gramm-Mol NaSH pro Mol Schwefelhalogenid in einem wäßrigen Alkoholmedium bei einer Temperatur von 50_{°}C bis zu Rückfluß zur Bildung des sulfurierten Olefins umsetzt,
(C) das sulfurierte Olefin aus dem wäßrigen Alkoholmedium abtrennt.

6. Sulfuriertes Olefin nach Anspruch 5 und weiter durch die Merkmale eines oder mehrerer Ansprüche 2 bis 4 definiert.

7. Schmierölzusammensetzung, enthaltend eine Hauptmenge aus einem Öl mit Schmierviskosität, enthaltend eine kleinere, die Hochdruckeigenschaften verbessernde Menge eines sulfurierten Olefins gemäß Anspruch 5 oder Anspruch 6.

8. Schmierölzusammensetzung nach Anspruch 7, worin das Olefin Isobutylen ist, das Schwefelhalogenid S₂CI₂ und das Alkylmercaptan tert-Butylmercaptan ist.

9. Verfahren zur Herstellung einer Zusammensetzung, bei dem man in ein Grundöl oder Kohlenwasserstoffflüssigkeit ein sulfuriertes Olefin nach Anspruch 5 oder 6 einmischt, um entweder eine Zusammensetzung nach Anspruch 7 oder eine Additivmenge oder -konzentrat herzustellen, worin die Menge des Olefins die kleinere Menge die Hochdruckeigenschaften verbessernde Menge übersteigt, wobei die Additivmenge für die anschließende Weiterverdünnung mit einem Schmieröl geeignet ist, um eine Schmierölzusammensetzung mit hochdruckresistenten Eigenschaften herzustellen.

## Revendications

1. Procédé de production d'une oléfine sulfurée de solubilité renforcée dans une huile lubrifiante, procédé caractérisé en ce qu'il consiste:
(A) à faire réagir un halogénure de soufre choisi entre S₂CI₂ et SCI₂ avec une mono-oléfine aliphatique contenant 3 à 6 atomes de carbone pour former un produit d'addition,
(B) à faire réagir ledit produit d'addition avec du soufre, Na₂S, en une quantité de 0,5 à 2,0 molécules- grammes par mole de chlorure de soufre, un alkyl-mercaptan contenant 1 à 12 atomes de carbone et 0 à 0,5 molécule-gramme de NaSH par mole d'halogénures de soufre dans un milieu alcoolique aqueux à une température allant de 50_{°}C à la température de reflux pour former ladite oléfine sulfurée,
(C) à séparer cette oléfine sulfurée du milieu alcoolique aqueux.

2. Procédé suivant la revendication 1, dans lequel ledit halogénure de soufre est 8₂0)₂.

3. Procédé suivant la revendication 2, dans lequel ladite mono-oléfine est une mono-oléfine à chaîne ramifiée ayant 4 à 6 atomes de carbone.

4. Procédé suivant la revendication 3, dans lequel ladite mono-oléfine est l'isobutylène.

5. Oléfine sulfurée pouvant être utilisée comme additif d'extrême-pression dans une huile lubrifiante ayant une solubilité renforcée, ladite oléfine sulfurée étant le produit préparé par un procédé qui consiste:
(A) à faire réagir un halogénure de soufre choisi entre S₂CI₂ et SC1₂ avec une mono-oléfine aliphatique contenant 3 à 6 atomes de carbone pour former un produit d'addition,
(B) à faire réagir ledit produit d'addition avec du soufre, Na₂S, en une quantité de 0,5 à 2,0 molécules- grammes par mole de chlorure de soufre, un alkyl-mercaptan contenant 1 à 12 atomes de carbone et 0 à 0,5 molécule-gramme de NaSH par mole d'halogénure de soufre dans un milieu alcoolique aqueux à une température allant de 50_{°}C à la température de reflux pour former ladite oléfine sulfurée,
(C) à séparer cette oléfine sulfurée du milieu alcoolique aqueux.

6. Oléfine sulfurée suivant la revendication 5, définie en outre par les particularités de l'une quelconque ou plusieurs des revendications 2 à 4.

7. Composition d'huile lubrifiante comprenant une quantité dominante d'une huile de viscosité propre à la lubrification, contenant une quantité secondaire améliorant les propriétés d'extrême-pression d'une oléfine sulfurée suivant la revendication 5 ou la revendication 6.

8. Composition d'huile lubrifiante suivant la revendication 7, dans laquelle ladite oléfine est l'isobutylè- ne, ledit halogénure de soufre est S₂S1₂ et ledit alkyl-mercaptan est le tertio-butyl-mercaptan.

9. Procédé de production d'une composition, qui consiste à incorporer par mélange dans une huile de base ou dans un liquide hydrocarboné une oléfine sulfurée suivant la revendication 5 ou la revendication 6 de manière à produire ou bien une composition suivant la revendication 7 ou bien un additif conditionné ou un concentré d'additif dans lequel la quantité de ladite oléfine dépasse ladite quantité secondaire améliorant l'extrême-pression, après quoi ledit additif conditionné convient pour une dilution ultérieure avec une huile lubrifiante de manière à produire une composition d'huile lubrifiante douée de propriétés de résistance à la pression.
